

Jan. 30, 1951

C. C. LARSON

2,539,442

PROCESS OF PREPARING A DOUBLE-SIDED MOSAIC ELECTRODE

Filed July 1, 1946

FIG. 2



FIG. 3



FIG. 4



FIG. 5



FIG. 6



FIG. 7



FIG. 8



FIG. 9



FIG. 1

INVENTOR  
CHRISTIAN C. LARSON

BY 

ATTORNEY

## UNITED STATES PATENT OFFICE

2,539,442

## PROCESS OF PREPARING A DOUBLE-SIDED MOSAIC ELECTRODE

Christian C. Larson, Fort Wayne, Ind., assignor,  
by mesne assignments, to Farnsworth Research  
Corporation, a corporation of Indiana

Application July 1, 1946, Serial No. 680,798

15 Claims. (Cl. 204—24)

1

This invention relates to electrodes for television tubes and particularly to a novel process of preparing a double-sided mosaic electrode for use in certain types of picture analyzing devices.

A double-sided mosaic electrode may be arranged in a picture signal generating tube of the charge storage type in such a manner as to have an optical image of the object projected upon one of its surfaces, while its opposite surface is scanned by an electron beam for developing picture signals. It is well known in the art that a double-sided mosaic electrode will appreciably improve the performance of picture signal generating tubes of the charge storage type. It is feasible, for example, to provide an accelerating electrode opposite the photosensitive surface of the mosaic for collecting the photoelectrons which are liberated from the mosaic by the action of the light. This will increase the signal output of the tube by saturating the photoemission and improve the signal-to-noise ratio. Furthermore, the scanning beam which may be arranged to the rear of the mosaic electrode may have a common axis with the optical system provided for imaging the object on the mosaic electrode. Thus, the so-called keystone effect is eliminated which is caused in a conventional picture analyzing tube of the cathode ray type by the necessity to arrange the scanning beam at an acute angle with respect to the mosaic electrode. An appreciable improvement of the signal-to-noise ratio of the image orthicon may also be expected by utilizing a double-sided mosaic electrode therein.

Numerous attempts have been made to provide a double-sided mosaic electrode which essentially consists of an insulating sheet or foil having a multitude of metallic plugs extending therethrough and insulated from each other. Thus, it has been suggested to provide a wire screen with an insulating layer and to fill the interstices of the insulated screen with a paste of a metal oxide suspended in a binder which is thereafter heated to reduce the oxide and evaporate the binder of the paste. However, since the thickness of the wire screen is of the order of .001 inch, it is obviously extremely difficult to fill the very small interstices in the wire screen uniformly with a metallic paste. It has also been suggested to electroplate a metal onto a continuous conductor provided on one of the surfaces of the insulated wire screen, thereby to fill the interstices of the screen with metallic plugs. However, the difficulties of removing this conductor again, such as by grinding, are appreciable. Furthermore, the thus ap-

2

plied metal will normally not adhere to the walls of the interstices of the insulated wire screen so that the metallic plugs are liable to fall out.

It is the principal object of the present invention, therefore, to provide a novel process of preparing a double-sided mosaic electrode suitable for use in cathode ray television transmitting tubes.

A further object of the invention is to provide a simple and convenient method of preparing a double-sided mosaic electrode adapted for use in a picture analyzing device for the transmission of television pictures of high definition.

In accordance with the present invention, the process of preparing a double-sided mosaic electrode from a fine mesh metallic screen comprises the steps of coating the screen with an electrically insulating substance, and then coating one face of the screen and the inner walls 20 of the interstices thereof with an electrically conducting material. The face of the screen coated with the conducting material is now covered with a removable insulating layer, and the interstices of the screen are filled with a metal 25 by electroplating it onto the conducting material, that is, onto the conducting material on the inner walls of the interstices. Finally the insulating layer and the conducting material are removed from the face of the screen coated therewith.

For a better understanding of the invention, together with other and further objects thereof, reference is made to the following description, taken in connection with the accompanying drawing, and its scope will be pointed out in the appended claims.

In the accompanying drawing:  
Fig. 1 is a plan view on greatly enlarged scale of a fragmentary portion of a very fine mesh 40 metallic screen utilized as a base of a double-sided mosaic electrode in accordance with the invention;

Fig. 2 is a sectional view taken on line 2—2 of Fig. 1 of the fine mesh metallic screen;

Figs. 3 to 9 are sectional views similar to Fig. 2 illustrating consecutive steps in the process of preparing a double-sided mosaic electrode in accordance with the present invention;

Fig. 3 illustrates the screen coated with a 50 reinforcing metallic layer;

Fig. 4 illustrates the screen of Fig. 3 provided with an insulating substance;

Fig. 5 illustrates the screen of Fig. 4 covered on one of its faces and on the inner walls of its 55 interstices with a conducting material;

Fig. 6 illustrates the screen of Fig. 5 covered

on its metal coated surface with an insulating layer applied thereto by a glass plate;

Fig. 7 illustrates the screen of Fig. 6 provided with metallic plugs in the interstices of the screen;

Fig. 8 illustrates the screen of Fig. 7 with the insulating layer removed; and

Fig. 9 illustrates the screen of Fig. 8 with the conducting material removed from the face of the screen, the screen being now ready for use.

Referring to the drawing, there is shown in Figs. 1 and 2 a very fine mesh metallic screen 1 which may, for example, consist of copper. Metallic screen 1 is provided with a multiplicity of apertures or interstices 2 which preferably are of circular shape as illustrated in Fig. 1. Metallic screen 1 may be an 800 or 1,000 mesh screen, that is, there are 800 or 1,000 holes per linear inch, respectively, corresponding to 640,000 holes or 1,000,000 holes per square inch. Thus, the number of interstices 2 is so large that at least three and preferably four interstices or holes are covered by any picture element in a conventional picture analyzing tube of the cathode ray type. Screen 1 may have a thickness of .0001 inch. Alternatively, screen 1 may consist of a very fine mesh wire screen instead of a very fine mesh perforated metallic sheet or foil.

Metallic screen 1 may now be covered as shown in Fig. 3 with a reinforcing metallic layer 3 which may be applied, for example, by evaporation. Metallic layer 3 covers both faces of screen 1 as well as the inner walls of interstices 2. Metallic layer 3 may, for example, consist of gold for a purpose to be explained hereinafter. However, it is to be understood that it is not necessary to coat screen 1 with a metallic layer such as 3.

Metallic screen 1 which may or may not be covered with metallic layer 3 is now coated with an electrically insulating substance indicated at 4 in Fig. 4 which covers the entire surface of screen 1 including the inner walls of interstices 2. Insulating substance 4 may consist, for example, of calcium fluoride or silicon oxide. Thus, insulating substance 4 may be applied, for example, by evaporating quartz onto metallic screen 1 in such a manner that the entire surface thereof is covered with a quartz layer. Screen 1 is now electrically insulated.

The thus insulated metallic screen 1 is then coated with an electrically conducting material 5, such as copper which may be dissolved with an acid, or with aluminum which may be dissolved with an alkaline hydroxide including sodium hydroxide and potassium hydroxide. Conducting material 5 is applied, such as by evaporation, to face 6 of screen 1 and to the inner walls of interstices 2 as shown in Fig. 5. Accordingly, the opposite face of metallic screen 1 is free from conducting material 5 so that insulating substance 4 is uncovered.

Face 6 of metallic screen 1 which has previously been coated with electrically conducting material 5 is now covered with a removable insulating layer indicated at 7 in Fig. 6. Removable insulating layer 7 may, for example, consist of a lacquer which may be pressed against face 6 of screen 1 by glass plate 8. Thus, conducting material 5 on face 6 of screen 1 is entirely covered by insulating layer 7 while the conducting material 5 is still exposed in the inner walls of interstices 2.

Conducting material 5 on the inner walls of interstices 2 which may consist of copper or

aluminum as pointed out hereinbefore, may be used in accordance with the present invention as an electrode for filling interstices 2 with a metal 10 which is electroplated onto conducting material 5.

Conducting material 5 on face 6 of screen 1 is covered by insulating layer 7 so that metal 10 cannot be deposited thereon. As shown in Fig. 7, interstices 2 are filled by metallic plugs 10 which may, for example, consist of gold or platinum, that is, of any metal which is resistant against acids or bases. Electrical contact may be made to conducting material 5 on the inner walls of interstices 2 from face 6 of screen 1. Metallic plugs 10 will strongly adhere to conducting material 5 on the inner walls of interstices 2.

The exposed faces of metallic plugs 10 may be provided at this stage with caps 11 by electroplating a metal, such as silver thereon, which may be made photosensitive in accordance with conventional practice. Electrical contact for the electrodeposition of caps 11 may be made again through metallic plugs 10 to conducting material 5 on face 6 of screen 1.

Insulating layer 7 and glass plate 8 are now removed by dissolving layer 7 in a suitable solvent, and the resulting screen is illustrated in Fig. 8. Accordingly, conducting material 5 on face 6 of screen 1 is exposed again.

The last step of the process of the invention consists in removing conducting material 5 from face 6 of screen 1. If conducting material 5 consists, for example, of copper, it may be removed by a suitable acid such as nitric acid, sulphuric acid or hydrochloric acid, which will not dissolve metallic plugs 10 which may consist of gold or platinum. Caps 11 may consist of a silver layer of such a thickness that the silver will not be dissolved before copper layer 5 on face 6 of screen 1 has been entirely dissolved. Alternatively, conducting material 5 may consist of aluminum. In that case aluminum layer 5 exposed on face 6 of screen 1 may be dissolved by sodium hydroxide or potassium hydroxide. Metallic plugs 10 should consist of a material such as gold or platinum which is resistant to the alkaline hydroxide used for dissolving aluminum layer 5.

It is to be understood that caps 11 need not be provided in case metallic plugs 10 consist of gold because gold may also be made photosensitive.

The finished screen is illustrated in Fig. 9 and consists of a multiplicity of metallic plugs 10 insulated from each other by insulating substance 4. One of the faces of metallic plugs 10 may be made photosensitive in order to develop an electrical charge image when light image is projected thereon. The reverse face of screen 1, which may be face 6, may then be scanned by an electron beam for developing picture signals.

Reinforcing metallic layer 3 which may consist of gold further serves the purpose of protecting screen 1 which may consist of a base metal, such as copper, from the action of the acid or the alkaline hydroxide utilized for removing the exposed portion of conducting material 5. Thus, the acid or base may dissolve metallic screen 1 through pin holes or cracks in insulating substance 4 which normally would protect metallic screen 1 from the action of the acid or base. Since the thickness of metallic screen 1 is of the order of .0001 inch, a base metal such as copper will be dissolved almost instantly by an acid if it is not protected over its entire surface by insulating substance 4.

While there has been described what is at present considered the preferred embodiment of the invention, it will be obvious to those skilled in the art that various changes and modifications may be made therein without departing from the invention, and it is, therefore, aimed in the appended claims to cover all such changes and modifications as fall within the true spirit and scope of the invention.

What is claimed is:

1. The process of preparing a double-sided mosaic electrode from a fine mesh metallic screen which comprises coating said screen with an electrically insulating substance, coating one face of said screen and the inner walls of the interstices thereof with an electrically conducting material, covering the face of said screen coated with said conducting material with a removable insulating layer, filling said interstices with a metal by electroplating it onto said conducting material, and removing said insulating layer and said conducting material from the face of said screen coated therewith.

2. The process of preparing a double-sided mosaic electrode from a fine mesh metallic screen which comprises coating said screen with an electrically insulating substance, coating one face of said screen and the inner walls of the interstices thereof with an electrically conducting material, covering the surface of said screen coated with said conducting material with a removable insulating layer, filling said interstices with a metal by electroplating it onto said conducting material, electroplating onto one of the exposed surfaces of said metal in said interstices a substance which may be photosensitized, and removing said insulating layer and said conducting material from the face of said screen coated therewith.

3. The method of preparing a double-sided mosaic electrode from a fine mesh metallic screen which comprises coating said screen with a metallic layer, coating said metallic layer with an electrically insulating substance, thereafter coating one face of said screen and the inner walls of the interstices thereof with an electrically conducting material, covering the face of said screen coated with said conducting material with a removable insulator, filling said interstices with a metal by electroplating it onto said conducting material on said inner walls, and removing said insulator and said conducting material from the face of said screen coated therewith.

4. The method of preparing a double-sided mosaic electrode from a fine mesh metallic screen which comprises coating said screen with a metallic layer, coating said metallic layer with an electrically insulating substance, thereafter coating one face of said screen and the inner walls of the interstices thereof with an electrically conducting material, covering the face of said screen coated with said conducting material with a removable insulator, filling said interstices with a metal by electroplating it onto said conducting material on said inner walls, electroplating onto one of the exposed surfaces of said metal in said interstices a substance which may be photosensitized, and removing said insulator and said conducting material from the face of said screen coated therewith.

5. The method of preparing a double-sided mosaic electrode from a fine mesh metallic screen which comprises coating said screen with an electrically insulating substance, thereafter coating one face of said screen and the inner walls of the interstices thereof with a first metal

which may be dissolved by a predetermined solvent, covering the face of said screen coated with said first metal with a removable insulating layer, filling said interstices with a second metal which is substantially not dissolved by said solvent by electroplating it onto said first metal on said inner walls, removing said insulating layer, and removing said first metal from the face of said screen coated therewith by dissolving it with said solvent.

6. The method of preparing a double-sided mosaic electrode from a fine mesh metallic screen which comprises coating said screen with a material which is resistant to a predetermined solvent, coating said material with an electrically insulating substance, thereafter coating one face of said screen and the inner walls of the interstices thereof with a first metal which may be dissolved by said solvent, covering the face of said screen coated with said first metal with a removable insulating layer, filling said interstices with a second metal which is substantially not dissolved by said solvent by electroplating it onto said first metal on said inner walls, removing said insulating layer, and removing said first metal from the face of said screen coated therewith by dissolving it with said solvent.

7. The method of preparing a double-sided mosaic electrode from a fine mesh metallic screen which comprises coating said screen with a material which is resistant to a predetermined solvent, coating said material with an electrically insulating substance, thereafter coating one face of said screen and the inner walls of the interstices thereof with a first metal which may be dissolved by said solvent, covering the face of said screen coated with said first metal with a removable insulating layer, filling said interstices with a second metal which is substantially not dissolved by said solvent by electroplating it onto said first metal on said inner walls, electroplating onto one of the exposed surfaces of said second metal in said interstices a substance which may be photosensitized, removing said insulating layer, and removing said first metal from the face of said screen coated therewith by dissolving it with said solvent.

8. The process of preparing a double-sided mosaic electrode from a fine mesh metallic screen which comprises coating said screen with an electrically insulating substance, thereafter coating one face of said screen and the inner walls of the interstices thereof with a first metal which may be dissolved by a predetermined acid, covering the face of said screen coated with said metal with a removable insulating layer, filling said interstices with a second metal which is not dissolved by said acid by electroplating it onto said first metal on said inner walls, removing said insulating layer, and removing said first metal from the face of said screen coated therewith by dissolving it with said acid.

9. The process of preparing a double-sided mosaic electrode from a fine mesh metallic screen which comprises coating said screen with a first metal resistant to a predetermined acid, coating said metal with an electrically insulating substance, thereafter coating one face of said screen and the inner walls of the interstices thereof with a second metal which may be dissolved by said acid, covering the face of said screen coated with said second metal with a removable insulating layer, filling said interstices with a metal which is not dissolved by said acid by electroplating it onto said second metal on said inner

walls, removing said insulating layer, and removing said second metal from the face of said screen coated therewith by dissolving it with said acid.

10. The process of preparing a double-sided mosaic electrode from a fine mesh metallic screen which comprises coating said screen with an electrically insulating substance, thereafter coating one face of said screen and the inner walls of the interstices thereof with copper, covering the face of said screen coated with said copper with a removable insulating layer, filling said interstices with gold by electroplating it onto said copper on said inner walls, removing said insulating layer, and removing said copper from the face of said screen coated therewith by dissolving it with an acid.

11. The process of preparing a double-sided mosaic electrode from a fine mesh metallic screen which comprises coating said screen with gold, coating said gold with an electrically insulating substance, thereafter coating one face of said screen and the inner walls of the interstices thereof with copper, covering the face of said screen coated with said copper with a removable insulating layer, filling said interstices with gold by electroplating it onto said copper on said inner walls, removing said insulating layer, and removing said copper from the face of said screen coated therewith by dissolving it with an acid.

12. The method of preparing a double-sided mosaic electrode from a fine mesh metallic screen which comprises coating said screen with an electrically insulating substance, thereafter coating one face of said screen and the inner walls of the interstices thereof with a base metal which may be dissolved by a predetermined alkaline hydroxide, covering the face of said screen coated with said base metal with a removable insulating layer, filling said interstices with a noble metal which is not dissolved by said alkaline hydroxide by electroplating it onto said base metal on said inner walls, removing said insulating layer, and removing said base metal from the face of said screen coated therewith by dissolving it with said alkaline hydroxide.

13. The method of preparing a double-sided mosaic electrode from a fine mesh metallic screen which comprises coating said screen with a metallic layer resistant to a predetermined alkaline hydroxide, coating said metallic layer with an electrically insulating substance, thereafter coating one face of said screen and the inner walls of the interstices thereof with a base metal which may be dissolved by said alkaline hydroxide, covering the face of said screen coated with said base metal with a removable insulating layer, filling said interstices with a noble metal which

is not dissolved by said alkaline hydroxide by electroplating it onto said base metal on said inner walls, removing said insulating layer, and removing said base metal from the face of said screen coated therewith by dissolving it with said alkaline hydroxide.

14. The method of preparing a double-sided mosaic electrode from a fine mesh metallic screen which comprises coating said screen with an electrically insulating substance, thereafter coating one face of said screen and the inner walls of the interstices thereof with aluminum, covering the face of said screen coated with said aluminum with a removable insulating layer filling said interstices with gold by electroplating it onto said aluminum on said inner walls, removing said insulating layer, and removing said aluminum from the face of said screen coated therewith by dissolving it with an alkaline hydroxide.

15. The method of preparing a double-sided mosaic electrode from a fine mesh metallic screen which comprises coating said screen with a gold layer, coating said gold layer with an electrically insulating substance, thereafter coating one face of said screen and the inner walls of the interstices thereof with aluminum, covering the face of said screen coated with said aluminum with a removable insulating layer, filling said interstices with gold by electroplating it onto said aluminum on said inner walls, removing said insulating layer, and removing said aluminum from the face of said screen coated therewith by dissolving it with an alkaline hydroxide.

CHRISTIAN C. LARSON.

#### REFERENCES CITED

The following references are of record in the file of this patent:

#### UNITED STATES PATENTS

| Number    | Name            | Date          |
|-----------|-----------------|---------------|
| 577,070   | Sandham         | Feb. 16, 1897 |
| 997,610   | Feldkamp        | July 11, 1911 |
| 1,243,654 | Clark           | Oct. 16, 1917 |
| 1,323,167 | Denny           | Nov. 25, 1919 |
| 1,792,197 | Stresau         | Feb. 10, 1931 |
| 2,045,984 | Flory           | June 30, 1936 |
| 2,047,369 | Hickok          | July 14, 1936 |
| 2,182,578 | Blumlein et al. | Dec. 5, 1939  |
| 2,217,334 | Diggory         | Oct. 8, 1940  |
| 2,226,384 | Vorris          | Dec. 24, 1940 |

#### FOREIGN PATENTS

| Number  | Country       | Date          |
|---------|---------------|---------------|
| 335,161 | Great Britain | Apr. 14, 1930 |
| 524,354 | Great Britain | Aug. 5, 1940  |